

## 1

3,552,983

**FOUNDRY SAND COMPOSITIONS**

 John V. Phillips, 248 Voss Road,  
 Bethel Park, Pa. 15102

 No Drawing. Filed July 30, 1969, Ser. No. 846,288  
 Int. Cl. B28b 7/34

U.S. Cl. 106—38.35

4 Claims

**ABSTRACT OF THE DISCLOSURE**

A foundry mold and core sand composition is provided made up of Chromite Sand, Chromite Sand Flour, Bentonite, Cereal Binder and water which composition may be stored for extended periods of time in the mixed condition without deterioration and which may be used for patching, for the formation of intricate molds and cores and for any other use to which foundry sand composition are conventionally used.

This invention relates to foundry sand compositions and particularly to a water base sand molding composition which may be stored and yet will dry rapidly when used and exposed to the air.

The problems of finding a sand composition for foundry use which will take intricate shapes, can be stored wet, and yet can be rammed and oven dried to get clean casting without expensive chipping are problems which have been the object of considerable research in the foundry industry for many years. There have, over the years, been developed many binders and sand formulations for making cores and molds. Historically, molds and cores are formed by mixing sands of various types and binders and drying same principally by using large heated, drying furnaces. This practice is time consuming and expensive. There have been more recently developed a variety of binders which can be used with sands to eliminate the use of the heating furnaces for drying and the resulting cores and molds can be air dried to produce a satisfactory resultant core or mold. These materials are based on resinous primers such as urea furfuryl alcohol formaldehyde and the like materials. They depend upon a polymerization reaction for their usefulness. Once mixed, they have a very short storage life, and they are subject to many problems in use. There has long been a need for a foundry composition which could be premixed, stored for several days, and used as needed without any problem of early set up. Such composition is particularly advantageous for making cores, highly intricate parts and for patching cores and molds which have been made using conventional drying oil binders. The present invention provides just such a foundry composition.

I have developed a foundry sand composition which is water based and does not use any of the polymerizable drying oils as a binder. It may be premixed and stored for a week or more under proper conditions. The core or mold when dried, is extremely hard making it easy to handle, and because of its quality, intricate shapes can be made at a minimum thickness while core breakage is kept to a minimum.

I provide a foundry sand composition which in its broadest range has the following makeup:

About 150 lbs.—225 lbs. of Chromite Sand (A.F.A. Grain Fineness No. 80)

About 75 lbs.—150 lbs. Chromite Sand Flour (A.F.A. Grain Fineness No. 325)

About 3 lbs.—5 lbs. of Western Bentonite

About 1/2 lbs.—2 lbs. of Corn Cereal Binder

The foregoing composition is mixed with sufficient moisture to provide a handleable and formable mix-

## 2

ture. This will amount to about 2 1/2 gallons of water in the above amount of sand composition. While the foregoing broad general range of material will produce the desired results, I prefer the following narrower composition.

- 5      200 lbs. Chromite Sand (A.F.A. Grain Fineness No. 80)  
 100 lbs. Chromite Sand Flour (A.F.A. Grain Fineness No. 325)  
 10     3 1/2 lbs. (2 qt.) Western Bentonite  
 15     1 lb (1 qt.) Mogul. (Corn Cereal Binder) to which is added sufficient water to make the mixture formable. The preferred amount is about 2 1/2 gallons. The mixture is mulled for about 2 1/2 minutes and formed into the desired cores and molds. The product resulting from the foregoing narrow composition will have the following grain fineness.

**GRAIN FINENESS**

|    | U.S. Sieve No. | Percent |
|----|----------------|---------|
| 20 | 30             | 0.2     |
|    | 40             | 1.0     |
|    | 50             | 6.0     |
|    | 70             | 12.6    |
| 25 | 100            | 17.1    |
|    | 140            | 12.6    |
|    | 200            | 8.0     |
|    | 270            | 3.0     |
|    | Pan            | 39.5    |

30 The general physical characteristics of the composition are:

- Sand Analysis  
 35     Moisture—5.5—6.0%  
 Green compression—8.5—9.0 p.s.i.  
 Green permeability—8—10  
 Dry shear—73 plus (p.s.i.)  
 Grain fineness number—165—175 (170 average)  
 2" specimen—320 grams

40 Compositions made according to the above described mixture when mulled with water only, have been packaged in polyethylene bags and stored for as much as seven weeks with test cores being made everyday with the production of very satisfactory cores even on the seventh week with no indicated deterioration in the mixture.

45 The composition of this invention can be used throughout the foundry in any troublesome areas of molds or cores with the elimination of conventional oil binders and oil sand compositions. The mixture is particularly advantageous in patching damaged core or mold sections. For example, a core which has had a portion broken away may be patched by applying a light coat of good

50 grade ceramic base core paste (water soluble) to the damaged area and drying it until tacky. The composition of the present invention is then applied and rammed firmly. The patched area is then permitted to dry. The resulting patched core will show no parting line at the patched area.

60 The composition is very useful for patching lift hook holes on the metal face of cores and for the variety of other purposes which had heretofore been very difficult to handle. The composition of this invention can be dried at any normal oven temperature from 375° F. and up. However, as has been pointed out, it will air dry rapidly on small patched areas and can be used as patching on any of the conventional foundry sand core oil compositions. The range of compositions which I have set out in this particular application is one

65 which defines a composition highly useful for solving problem areas in forming molds and cores. The outside limits are critical. If the composition is altered outside

the limits here disclosed, the composition becomes too brittle on the one hand, and on the other hand, there is insufficient binding effect to hold the material together so that it is imperative that the composition be held within the broad range here set out.

While I have disclosed a preferred practice and embodiments of this invention, it will be understood that the invention will be otherwise embodied within the scope of the following claims.

I claim:

1. A foundry sand composition consisting essentially of 150 lbs.-250 lbs. of Chromite Sand, about 75 lbs.-150 lbs. of Chromite Sand Flour, about 3 lbs.-5 lbs. of Bentonite, about 1/2-2 lbs. of Cereal Binder, and sufficient water to make a formable mixture.

2. A composition for foundry sand cores and molds as claimed in claim 1 wherein the Cereal Binder is Corn Cereal Binder.

3. A composition as claimed in claim 1 wherein there is provided 200 lbs. of Chromite Sand, 100 lbs. of Chromite Sand Flour, 3 1/2 lbs. of Bentonite, 1 1/2 lbs. of Corn

Cereal Binder, and sufficient water to form a mixture which may be formed and set.

4. A composition as claimed in claim 1 wherein the Chromite Sand has a grain fineness in the A.F.A. of 80, and the Chromite Sand Flour has a grain fineness A.F.A. 325.

#### References Cited

##### UNITED STATES PATENTS

|           |        |                  |            |
|-----------|--------|------------------|------------|
| 2,504,133 | 4/1950 | Kerlin           | 106-38.5X  |
| 2,790,218 | 4/1957 | Kohl et al.      | 106-38.35X |
| 2,798,817 | 7/1957 | Lund             | 106-38.23  |
| 2,830,913 | 4/1958 | Meyers et al.    | 106-38.9   |
| 3,146,113 | 8/1964 | Middleton et al. | 106-38.23  |

15 LORENZO B. HAYES, Primary Examiner

U.S. CL. X.R.

106-38.3, 38.5, 66, 71

20